

Nov. 12, 1935.

R. SCHNEIDEWIND

2,020,382

CHROMIUM PLATING

Filed June 13, 1934



Richard Schneidewind

Charles H. Field  
ALTS

## UNITED STATES PATENT OFFICE

2,020,382

## CHROMIUM PLATING

Richard Schneidewind, Ann Arbor, Mich.

Application June 13, 1934, Serial No. 730,427

15 Claims. (Cl. 204—1)

This invention relates to a method for increasing the throwing power and utility of a chromium plating bath.

More specifically this invention relates to chromic acid plating baths of superior throwing powers which have an agent incorporated therein capable of reducing the normal lower limit of the current density of the bath.

In my copending application entitled "Method of chromium plating", Serial No. 687,414, filed August 30, 1933, I have described the effect of buffer agents such as boric acid in chromic acid plating baths. In this application I have shown results obtained by the incorporation of 20 grams or more of boric acid in a liter of chromic acid plating solution containing from 100 to 450 grams of  $\text{CrO}_3$  and from 0.5 to 6.2 grams of  $\text{SO}_4$ . The data in this application definitely proves that buffer agents such as boric acid and the like increase the upper limit of current density for plating articles with a bright chromium deposit.

I have now found that the incorporation of quinones, which are readily oxidized and reduced

the throwing power of a chromic acid plating bath by incorporating a quinone therein.

Another object of this invention is to provide a method for increasing the throwing power of chromic acid plating baths by incorporating quinones therein which are readily oxidized and reduced under the influence of electrolysis without interfering with the plating operation.

A further object of this invention is to provide a chromic acid plating bath of increased throwing power by incorporating hydroquinone therein.

Other and further objects of this invention will be apparent to those skilled in the art from the following specification and annexed sheet of drawing which forms a part of this specification.

On the drawing:

Figure 1 is a chart showing the effect of varying amounts of hydroquinone on the upper and lower limiting current densities in chromic acid plating baths containing 250 grams per liter of  $\text{CrO}_3$  and about 2.5 grams per liter of sulphate radicals ( $\text{SO}_4$ ). The curves were plotted from the following data:

| Hydroquinone grams per liter | Temp. 45° C.                                           |                          | CrO <sub>3</sub> =250 g/l    |  |
|------------------------------|--------------------------------------------------------|--------------------------|------------------------------|--|
|                              | Sulphate ratio, CrO <sub>3</sub> /SO <sub>4</sub> =100 |                          |                              |  |
|                              | Plating range                                          |                          |                              |  |
|                              | A                                                      | B                        | Throwing power $\frac{B}{A}$ |  |
|                              | Lower limit amp./sq. ft.                               | Upper limit amp./sq. ft. |                              |  |
| 0                            | 65                                                     | 205                      | 3.15 35                      |  |
| 0.1                          | 20                                                     | 196                      | 9.8                          |  |
| 0.2                          | 25                                                     | 200                      | 8.0                          |  |
| 0.25                         | 20                                                     | 200                      | 10.0                         |  |
| 0.5                          | 17                                                     | 205                      | 12.1                         |  |
| 1.0                          | 20                                                     | 206                      | 10.3                         |  |
| 2.0                          | 20                                                     | 200                      | 10.0                         |  |
| 5.0                          | 26                                                     | 175                      | 6.72 40                      |  |

under the influence of electrolysis, into a chromic acid plating bath decreases the necessary current density heretofore required for the production of bright plating. I have found that quinones such as benzoquinone, hydroquinone, naphthaquinone, anthraquinone and the like are operable for this purpose.

It is therefore an object of this invention to provide a chromium plating bath having increased throwing power especially in the lower ranges of current density used in the electrodeposition of chromium on metals for the production of bright plated surfaces thereon.

Another object of this invention is to increase

Figure 2 is a combined chart showing the effect of the change of sulphate ratio

$$\left( \frac{\text{CrO}_3}{\text{SO}_4} \right)$$

on the throwing power of chromic acid plating baths containing no hydroquinone and containing 0.5 grams per liter of hydroquinone. Curves 1 and 3 were obtained from plating operations carried out at 45° C. Curve 2 was obtained from data in plating operations carried out at 25° C. while curve 4 was obtained from data in plating operations effected at 60° C.

The data from which the curves were plotted in chart 2 is indicated in the following table:

treme tips also showed grayness. It should be appreciated that while only the upper and lower

| 5  | Hydroquinone g/l | Temper-<br>ature,<br>degrees<br>centigrade | CrO <sub>3</sub><br>SO <sub>4</sub> | Plating range               |                             | Throwing<br>power<br>$\frac{B}{A}$ |       |
|----|------------------|--------------------------------------------|-------------------------------------|-----------------------------|-----------------------------|------------------------------------|-------|
|    |                  |                                            |                                     | A                           | B                           |                                    |       |
| 10 |                  |                                            |                                     | Lower limit<br>amp./sq. ft. | Upper limit<br>amp./sq. ft. |                                    |       |
|    | 0                |                                            | 45                                  | 50                          | 170                         | 250                                | 1.47  |
|    | 0                |                                            | 45                                  | 65                          | 135                         | 195                                | 1.44  |
|    | Curve No. 1      | 0                                          | 45                                  | 100                         | 65                          | 205                                | 3.15  |
|    | 0                |                                            | 45                                  | 200                         | 65                          | 195                                | 3.0   |
|    | 0                |                                            | 45                                  | 300                         | 82                          | 190                                | 2.32  |
| 15 |                  |                                            |                                     |                             |                             |                                    | 10    |
|    | 0.5              |                                            | 25                                  | 50                          | 22                          | 111                                | 5.04  |
|    | 0.5              |                                            | 25                                  | 75                          | 18                          | 105                                | 5.82  |
|    | Curve No. 2      | 0.5                                        | 25                                  | 100                         | 5                           | 70                                 | 14.0  |
|    | 0.5              |                                            | 25                                  | 200                         | 13                          | 107                                | 8.2   |
|    | 0.5              |                                            | 25                                  | 300                         | 12                          | 88                                 | 7.33  |
| 20 |                  |                                            |                                     |                             |                             |                                    |       |
|    | 0.5              |                                            | 45                                  | 50                          | 39                          | 260                                | 6.67  |
|    | 0.5              |                                            | 45                                  | 75                          | 28                          | 190                                | 6.8   |
|    | Curve No. 3      | 0.5                                        | 45                                  | 100                         | 17                          | 205                                | 12.1  |
|    | 0.5              |                                            | 45                                  | 200                         | 28                          | 192                                | 6.85  |
|    | 0.5              |                                            | 45                                  | 300                         | 35                          | 195                                | 5.58  |
| 25 |                  |                                            |                                     |                             |                             |                                    |       |
|    | 0.5              |                                            | 60                                  | 50                          | 218                         | 500                                | 2.29  |
|    | 0.5              |                                            | 60                                  | 75                          | 175                         | 455                                | 2.78  |
|    | Curve No. 4      | 0.5                                        | 60                                  | 100                         | 35                          | 525                                | 15.00 |
|    | 0.5              |                                            | 60                                  | 200                         | 68                          | 506                                | 7.45  |
|    | 0.5              |                                            | 60                                  | 300                         | 78                          |                                    | 25    |

The chromic acid plating bath used in each instance contained 250 grams per liter of chromic acid ( $\text{CrO}_3$ ).  
30

35 Since it is always desirable to prepare a plating bath which can be used throughout a wide range of current densities it will be readily appreciated that the presence of a quinone such as hydroquinone is advantageous because, as shown in Figure 1, the quinone considerably lowers the lower limiting current density. The presence of even minute quantities of hydroquinone, for example 0.1 gram per liter reduces the lower limit 40 of the plating range from about 65 amperes per square foot to about 20 amperes per square foot. The upper limiting current density is not materially affected although chart 1 shows that the presence of considerable amounts of hydroquinone, i.e. 5 grams or more per liter, tends 45 to lower the upper limit.

The throwing power of the plating bath as indicated by the above tables is determined by dividing the upper limiting current density by the lower limiting current density.

The current densities were determined uniformly according to the following procedure. A cylindrical steel tank three inches in diameter and seven inches deep was connected electrically to act as an anode. Copper test strips one-half inch wide were immersed in the chromic acid solution in the tank to about three inches of their depth. The plating was conducted at temperatures of 25° C. (77° F.); 45° C. (113° F.) and 60° C. (140° F.). The strips were plated at varying current densities and the quality of the deposit on the strips was examined in diffused light. The time of plating was 120 seconds for the higher current densities and 180 seconds for the lower current densities.

66 A satisfactory plate was one which covered the specimen copper strip completely and brightly with no trace of dullness or turning at the tips. The upper and lower limits of the current densities were thus determined and it was also found that in some instances bright plating was obtained below the tabulated limiting current densities. However these data were rejected since traces of copper could be seen at the center 70 of the upper edge of the specimen. The ex-

limiting current densities are correlated in the above tables it was necessary to carry out from 5 to 15 separate tests to determine each upper and lower limit. 30

Chart 2 shows that the highest throwing powers of the chromic acid plating baths are obtainable with the standard Sargent solution containing 250 grams per liter of chromic acid ( $\text{CrO}_3$ ) and 2.5 grams per liter of sulphate radicals ( $\text{SO}_4$ ) giving a sulphate ratio of 100. However the presence of hydroquinone so greatly increases the throwing power of chromic acid plating baths that the sulphate ratio may be varied considerably from this amount without approaching the weaker throwing power of a chromic acid plating bath which does not contain a quinone. Thus at 45° C. satisfactory bright plating deposits were obtained with a sulphate ratio as high as 300. The bath had a throwing power of 5.58 as compared with 2.32 when no quinone was present in the bath.

Since hydroquinone, as indicated in the accompanying charts, materially decreases the lower limiting current density without substantially affecting the upper limiting current density, the presence of a quinone is highly desirable in plating operations where current density must be kept at a minimum. The lower current density, if desired, may be applied by "striking" i. e. applying a higher current for a short period of time, for example, about 10 seconds. If a plating bath not containing hydroquinone is "struck" slightly better covering is obtained in the low current density areas but unsatisfactory plate is obtained at each current density below 65 amperes per square foot at 45° C. whether it is "struck" or not. In the presence of hydroquinone, I have found that plating will take place at as low as 20 amperes per square foot at 45° C. Thus the hydroquinone seems to function as a depolarizer permitting deposition of chromium at approximately 0.2 volt lower than is possible in the absence of such material.

It is possible that the hydroquinone is oxidized by the chromic acid in the plating bath to quinhydrone. This latter material may react with hydrogen liberated at the cathode during the plating operation to reform hydroquinone. 75

This action of course may explain that the quinones act as depolarizers but I do not desire to be limited by any theory since it is possible that the presence of the substance has an entirely different chemical effect which is not at the present time understood.

I have found that the presence of one-half gram per liter of anthraquinone in a standard Sargent plating bath at 45° increases the throwing power from 3.17 to 3.72. The presence of one-half gram per liter of naphthaquinone increases the throwing power to 4.5. If one gram per liter of naphthaquinone is used in the plating bath, the throwing power is increased further to 6.62. The presence of 0.5 gram per liter of benzoquinone in the above mentioned plating bath increases the throwing power to 8.06.

From the above it is evident that a quinone has a decided beneficial effect upon chromic acid plating baths especially when the plating operation is carried out at low current densities. The quinone is apparently most beneficial in plating operations for the deposition of chromium directly on a copper surface. This copper surface need only be of minute thickness.

I am aware that numerous details of the process may be varied through a wide range without departing from the principles of this invention, and I, therefore, do not purpose limiting the patent granted hereon otherwise than necessitated by the prior art.

Having now described my invention, what I claim is:

1. The method of increasing the throwing power of chromium plating baths which comprises incorporating a quinone into said baths.

2. The method of increasing the throwing power of chromic acid plating baths having a sulphate ratio within the range of 50 to 300 which comprises incorporating small amounts of a quinone in the baths.

3. The method of increasing the throwing power of chromium plating baths containing about 250 grams per liter of chromic acid ( $\text{CrO}_3$ ) and about 2.5 grams per liter of sulphate radicals ( $\text{SO}_4$ ) which comprises incorporating in said baths an amount of a quinone equivalent to .05 to 5 grams per liter of hydroquinone.

4. The method of increasing the throwing power of standard chromic acid plating baths which comprises incorporating therein a depolarizer se-

lected from the group consisting of benzoquinone, hydroquinone, anthraquinone, and naphthaquinone.

5. The method of lowering the lower limiting current density in chromium plating operations which comprises dissolving hydroquinone into the chromic acid plating bath.

6. The method of chromium plating which comprises depositing chromium on a copper surface from a chromic acid plating bath containing small amounts of a quinone at current densities equivalent to below 65 amperes per square foot at 45° C.

7. The method of chromium plating which comprises depositing chromium on a copper surface from a chromic acid plating bath containing about 250 grams per liter of chromic acid ( $\text{CrO}_3$ ), about 2.5 grams per liter of sulphate radicals ( $\text{SO}_4$ ) and from 0.1 to 5 grams per liter of hydroquinone at current densities between 20 and 200 amperes per square foot at 45° C.

8. As a new composition, a plating bath containing chromic acid, sulphate radicals and small amounts of a quinone.

9. As a new composition, a plating bath containing chromic acid and sulphate radicals, the ratio  $\text{CrO}_3/\text{SO}_4$  being from 50 to 300, and containing from 0.1 to 5 grams per liter of a quinone.

10. The process of increasing the throwing power of chromic acid plating baths which comprises incorporating into said baths small amounts of anthraquinone.

11. The process of increasing the throwing power of chromic acid plating baths which comprises incorporating into said baths small amounts of naphthaquinone.

12. As a new composition, a plating bath containing chromic acid, sulphate radicals and small amounts of hydroquinone.

13. As a new composition, a plating bath containing chromic acid, sulphate radicals and small amounts of anthraquinone.

14. As a new composition, a plating bath containing chromic acid, sulphate radicals and small amounts of naphthaquinone.

15. As a new composition, a plating bath containing chromic acid and sulphate radicals, the ratio  $\text{CrO}_3/\text{SO}_4$  being from 50 to 300, and containing from 0.1 to 5 grams per liter of hydroquinone.

RICHARD SCHNEIDEWIND. 50